

## UNITED STATES PATENT OFFICE

2,642,397

## LUBRICATING GREASE COMPOSITIONS

Arnold J. Morway, Rahway, David W. Young, Roselle, and Delmer L. Cottle, Highland Park, N. J., assignors to Standard Oil Development Company, a corporation of Delaware

No Drawing. Application December 22, 1950.  
Serial No. 202,421

12 Claims. (Cl. 252—49.6)

1

This invention relates to novel lubricating grease compositions. Particularly, the invention relates to lubricating grease compositions prepared without the ordinary grease forming soaps. More particularly, the invention relates to new and useful lubricating grease compositions prepared by thickening a lubricating oil with an N-acyl amino phenol.

Lubricating engineers have long recognized the need for a lubricating grease composition which does not contain ash-forming soaps. There are many industrial uses for lubricating greases which will not leave deposited upon bearing surfaces the highly corrosive and frictional increasing soap residues when the grease composition has become volatilized.

It has now been found that lubricating oils may be thickened to form a grease composition by incorporating therein a minor amount of an N-acyl amino phenol wherein the acyl group contains from 14 to 22 carbon atoms per molecule.

These novel grease compositions have the advantage of leaving no soap residues on the bearing surfaces lubricated and, in addition, have the characteristic of being reversible, that is to say, the grease structure of these new lubricating compositions is not lost when the melting point is reached but rather on recrystallization, the thickening agent crystals redisperse to again form a stable grease structure.

The N-acyl amino phenols useful to form the non-soap grease compositions of this invention have the following general formula:



wherein R is an alkyl group containing from 14 to 22 carbon atoms, preferably an alkyl group which is non-benzenoid in nature, and wherein R' and R'' are hydrogen atoms or alkyl groups containing from 1 to 20 carbon atoms.

The preferred embodiment of this invention contemplates the use of compounds, according to the formula above, wherein R' and R'' are hydrogen atoms and wherein R is a straight chain aliphatic group containing from 14 to 22 carbon atoms. Exemplary of these preferred compounds are N-palmitoyl p-amino phenol, N-stearoyl p-amino phenol, and N-arachidoyl p-amino phenol, N-behenoyl p-amino phenol with the N-stearoyl or N-palmitoyl p-amino phenol or mixtures of each being especially preferred.

The alkylated acyl p-amino phenols exemplified by the formula above when R' and R'' are alkyl groups containing from 1 to 20 and pref-

erably from 4 to 15 carbon atoms, are also operable as lubricating oil thickeners. Compounds such as N-n-valeryl-4-amino-3-pentadecyl phenol, (N-n-pentanoyl-4-amino-3-pentadecyl phenol), N-n-propanoyl-4-amino-3-pentadecyl phenol, N-n-pentanoyl-4-amino-2,6-di-tert-butyl phenol, N-n-hexyl-4-amino-2-hexyl phenol, are examples of the alkylated acyl p-amino phenols which are operable.

The preparation of these acyl p-amino phenols is accomplished by simply admixing the desired acid or acid chloride with the desired p-amino phenol and heating the mixture under proper reaction conditions. The reaction progresses smoothly (splitting off water or hydrogen chloride) giving the desired amino phenol which may be purified by any of the various methods known to the art such as distillation, crystallization, extraction, etc.

To prepare the lubricating grease compositions of this invention, the desired acyl p-amino phenol is admixed with a lubricating oil in proportions varying from about 1% to about 10% by weight of the phenol to 99 to 90% by weight of the lubricating oil. The temperature is then raised to the melting point of the amino phenol and then allowed to cool to room temperature. During the process of cooling, the amino phenol recrystallizes in its dispersed state and causes the formation of a stable grease structure.

The oil selected to prepare the grease compositions of this invention may be widely varied. The oil chosen to prepare the grease for a particular lubricating use should be that oil which would be chosen if a liquid could be used in that particular lubricating operation. Mineral lubricating oils having viscosity ranges of from 55 to 2000 S. U. S. at 100° F. may be used depending upon the final formulation desired. The mineral oil may be of a paraffinic or naphthenic nature and may be a result of any of the well-known refining procedures.

A recent development in the lubricating art has been the adaptation for lubricating purposes of materials commonly known as "silicone oils." These silicone oils can be made by any of a variety of methods and very conveniently by reacting a Grignard reagent with a silicone halide, hydrolyzing the reaction product and then condensing with the elimination of water. The resulting siloxanes may then be polymerized into "silicone oils." Representative examples of these silicone oils may be mentioned polymers of methyl phenyl silicone, ethyl butyl silicone, methyl cyclo hexyl silicone, di-cyclo hexyl silicone, di-phenyl silicone, phenyl ethyl silicone, phenyl propyl silicone, and the like.

These silicone oils are generally inert, colorless, odorless liquids possessing an unusually low

rate of change of viscosity with temperature. The silicone oils remain permanent liquids over a wide range of temperatures, they are resistant to oxidation, and they are characterized by very low surface tensions. These silicone oils are substantially non-volatile at ordinary temperatures and exhibit extremely low pour points.

Grease compositions have been prepared using these silicone polymer oils by thickening them to grease structures with typical soap thickeners, lithium stearate being preferred. However, the common grease forming soaps, such as lithium stearate, cannot be dispersed directly in the silicone oils to form greases, but expensive and tedious methods of grease formation must be employed. Such methods include a pressurized solvent transfer.

It has been found, however, that these silicone polymer oils may be thickened to a grease consistency using the acyl p-amino phenols described above by a simple heating process. The greases so made contain all the advantageous properties expected from the use of the silicone polymer oil and, in addition, contain none of the soap residues heretofore experienced. Although any of the acyl p-amino phenols described above may be used to thicken the silicone oils, stearoyl p-amino phenol is preferred.

The preparation of these N-acyl amino phenols is accomplished by admixing the desired acid or acid chloride with the desired amino phenol and heating the mixture under proper reaction conditions. The reaction proceeds smoothly splitting off water or hydrogen chloride, giving the desired amino phenol as an end product. It may then be purified by any of the methods known to the art.

One method for the preparation of an operable p-amino phenol is typified by the following:

One mol of p-amino phenol was placed in a glass round bottomed flask fitted with a reflux condenser with an azeotropic take off arm. There was added to the flask one mol of stearic acid and about 150 cc. of xylene. The xylene served as an entraining agent for the water formed during the course of the reaction. The flask was then heated to the xylene reflux temperature and kept at that temperature for about 9 hours, or until 86% of the theoretical water (1 mol) had been removed. The contents of the flask was then emptied into an evaporating dish and heated on a steam bath until the last trace of xylene was removed. The product was then recrystallized from glacial acetic acid and there resulted a yield of 78% theoretical of colorless N-stearoyl p-amino phenol, melting point 132° C. Analysis for nitrogen was 3.75%, compared to a calculated 3.78%.

To more explicitly define the instant invention, the following examples are given:

#### EXAMPLE I

2.0% by weight of N-stearoyl p-amino phenol was admixed with 98.0% by weight of a Mid-Continent distillate having a viscosity at 210° F. of 56 S. U. S. and a viscosity index of 112. The mixture was heated with stirring to 275° F. at which point the amino phenol dissolved. The mixture was then allowed to cool to room temperature and a solid grease structure was obtained.

#### EXAMPLE II

3.5% N-stearoyl p-amino phenol was admixed with 96.5% of a solvent treated Mid-Continent distillate having a viscosity of 210° F. of 43

S. U. S. and a viscosity index of 112. The mixture was heated to 275° F. with stirring and then allowed to cool to room temperature. A translucent stable grease structure was obtained.

#### EXAMPLE III

Following the procedure detailed above an N-acyl p-amino phenol was prepared by reacting hydrogenated fish oil acids having carbon chain lengths ranging from C<sub>14</sub> to C<sub>22</sub> with p-amino phenol. 3.5% of this product was admixed with 96.5% of the oil used in Example II and the same procedure as in Example II was followed. There resulted a solid grease composition having excellent general appearance.

#### EXAMPLE IV

3.0% of N-erucyl p-amino phenol was admixed with 97% of a naphthenic base mineral oil having an S. U. S. viscosity at 100° F. of 500. The mixture was heated to 270° F. and the mass allowed to cool in pans. An excellent smooth grease was formed.

The greases of Examples I-IV were subjected to the standard ASTM penetration test after various amounts of working in a standard ASTM grease worker. The ASTM dropping point was also obtained. To determine the dispensability of the greases, they were subjected to a needle point fitting on a grease gun and were filtered through a 1,000 x 250 mesh metal screen. The results of these tests are set out in Table I below:

TABLE I  
Inspection data on mineral oil N-stearoyl p-amino phenol lubricating grease

|                                                   | Grease Sample |        |         |        |
|---------------------------------------------------|---------------|--------|---------|--------|
|                                                   | Ex. I         | Ex. II | Ex. III | Ex. IV |
| Penetration Data (mm./10 at 77° F.):              |               |        |         |        |
| Unworked.....                                     | 350           | 345    | 340     | 325    |
| Worked—                                           |               |        |         |        |
| 500 strokes (fine hole worker plate)              | 355           | 330    | 345     | 330    |
| 100,000 strokes (fine hole worker plate)          | 340           | 348    | 332     |        |
| Dropping Point (ASTM, °F.)                        | 240           | 245    | 245     | 245    |
| Water solubility (212° F./30 min.)                | nil           | nil    | nil     | nil    |
| Dispensability through needle point grease gun.   | good          | good   | good    | good   |
| Residue left on filtration through (1,000 X 250). | none          | none   | none    | none   |

#### EXAMPLE V

2.0% of N-stearoyl p-amino phenol was admixed with 98.0% of a phenyl methyl silicone polymer oil having a viscosity of 1000 S. U. S. at 100. The mixture was heated in a fire heated grease kettle with stirring to 275° F. and then allowed to cool in cooling pans to room temperature. A solid grease structure was obtained which was free from any oil separation.

Standard ASTM penetration data, ASTM dropping point, and water solubility tests are set out in Table II below:

In some instances it may be desirable to formulate a grease composition having a dropping point somewhat higher than that of Example V above. The addition of small amounts of lithium soap increases the dropping point of the grease of Example V to one in the neighborhood of 250° F. In this instance, however, the grease may not be prepared by simply mixing the ingredients. The lithium soap must first be dispersed in a mineral oil which dispersion is then incorporated into the silicone oil-amino phenol grease product. This is set out in detail in Example VI below.

## EXAMPLE VI

4.0% lithium stearate was dispersed in 10.0% of a refined mineral oil by heating to 400° F. with constant stirring. The mixture was then allowed to cool to 240° F. at which temperature 85.0% by weight of a phenyl methyl silicone polymer oil having a viscosity of 1000 S. U. S. at 100° F. was added. 1.0% of N-stearoyl p-amino phenol was added to the mixture and the mass then allowed to cool without further agitation. Inspection data on this lubricating grease are set out in Table III below:

TABLE III

Inspection data on grease of Example IV.

Penetration data (mm./10 at 77° F.):

|                                         |     |    |
|-----------------------------------------|-----|----|
| Unworked                                | 290 | 30 |
| Worked—                                 |     |    |
| 60 strokes (fine hole worker plate)     | 315 |    |
| 20,000 strokes (fine hole worker plate) | 345 |    |
| Dropping point (°F.)                    | 350 | 35 |
| Water solubility (30 min./212° F.)      | Nil |    |

By this method and combined use of the acyl p-amino phenol thickener, considerably less metallic soap is required to give a stable grease product of good yield. Any volatility of the mineral oil leaves a predominantly non-volatile grease. If desired, a volatile solvent may be replaced as the dispersant of the lithium soap under pressure and vaporized after the addition of the silicone fluid.

To recapitulate briefly, this invention is directed to new and useful grease compositions containing no soap prepared by thickening to a grease consistency a lubricating oil with from 1.5% to 5%, preferably 2.0% to 3.5% by weight, based on the total weight of the composition of a compound having the general formula



wherein R is an aliphatic group containing from 14 to 22 carbon atoms per molecule and R' and R'' are alkyl groups containing from 1 to 20 carbon atoms per molecule. The preferred grease compositions are prepared from the N-acyl p-amino phenols exemplified by N-palmitoyl p-amino phenol, N-stearoyl p-amino phenol, and N-arachidoyl p-amino phenol, with the stearoyl derivative being especially preferred. The grease compositions may be prepared using as a base oil either a refined mineral oil or a synthetic oil made by the polymerization of olefins, or a synthetic oil formed by polymerizing the so-called "silicones" commonly referred to as silicone polymer oils.

It is also within the concept of this invention to prepare the desired N-acyl p-amino phenol

in the lubricating oil to be used as the grease base. In this embodiment the calculated amount of the amino phenol is admixed with the oil and the desired acid or acid chloride is added drop-wise thereto.

It may be desired to add to the greases of this invention other of the well-known additive materials such as tackiness agents, corrosion inhibitors, oxidation inhibitors, detergents, and the like. This may be done with impunity in the greases of this invention since they are perfectly compatible with these additive materials.

What is claimed is:

1. A lubricating grease composition consisting essentially of a lubricating oil thickened to a grease consistency with a compound having the general formula



wherein R is an alkyl hydrocarbon group having from 14 to 22 carbon atoms and wherein R' and R'' are selected from the class consisting of hydrogen and alkyl groups containing from 1 to 20 carbon atoms.

2. A lubricating grease composition consisting essentially of a lubricating oil thickened to a grease consistency with a compound having the general formula



wherein R is an alkyl hydrocarbon group having from 14 to 22 carbon atoms and wherein R' and R'' are selected from the class consisting of hydrogen and alkyl groups containing from 4 to 15 carbon atoms.

3. A lubricating grease composition consisting essentially of a lubricating oil thickened to a grease consistency with a compound having the general formula



wherein R is an alkyl hydrocarbon group having 14 to 22 carbon atoms.

4. A lubricating grease composition consisting essentially of a lubricating oil thickened to a grease consistency with from 1% to 10% by weight based on the weight of the total composition of N-stearoyl p-amino phenol.

5. A lubricating grease composition consisting essentially of a mineral lubricating oil thickened to a grease consistency with from 1.5% to 5% by weight based on the weight of the total composition of N-stearoyl p-amino phenol.

6. A lubricating grease composition consisting essentially of a mineral lubricating oil thickened to a grease consistency with a compound having the general formula



wherein R is an alkyl hydrocarbon group having from 14 to 22 carbon atoms and wherein R' and R'' are selected from the class consisting of hydrogen and alkyl groups containing from 1 to 20 carbon atoms.

7. A lubricating grease composition consisting essentially of a mineral lubricating oil thickened to a grease consistency with a compound having the general formula



wherein R is an alkyl hydrocarbon group having from 14 to 22 carbon atoms and wherein R' and R'' are selected from the class consisting of hydrogen and alkyl groups containing from 4 to 15 carbon atoms.

8. A lubricating grease composition consisting essentially of a mineral lubricating oil thickened to a grease consistency with a compound having the general formula



9. A lubricating grease composition consisting essentially of a silicone polymer oil having a viscosity within a range of from 250 to 1000 S. U. S. at 100° F. thickened to a grease consistency with a compound having the general formula



wherein R is an alkyl hydrocarbon group having from 14 to 22 carbon atoms and wherein R' and R'' are selected from the class consisting of hydrogen and alkyl groups containing from 1 to 20 carbon atoms.

10. A lubricating grease composition consisting essentially of a polymer of methyl phenyl silicone having a viscosity of from 600 S. U. S. to 1000 S. U. S. at 100° F. thickened to a grease consistency with from 1.5% to 5% by weight based on the weight of the total composition of N-stearoyl p-amino phenol.

S. U. S. at 100° F. thickened to a grease consistency with a compound having the general formula



wherein R is an alkyl hydrocarbon group having from 14 to 22 carbon atoms and wherein R' and R'' are selected from the class consisting of hydrogen and alkyl groups containing from 1 to 20 carbon atoms.

11. A lubricating grease composition consisting essentially of a polymer of methyl phenyl silicone having a viscosity of from 600 S. U. S. to 1000 S. U. S. at 100° F. thickened to a grease consistency with a compound having the general formula



wherein R is an alkyl hydrocarbon group having 14 to 22 carbon atoms.

12. A lubricating grease composition consisting essentially of a polymer of methyl phenyl silicone having a viscosity of from 600 S. U. S. to 1000 S. U. S. at 100° F. thickened to a grease consistency with from 1.5% to 5% by weight based on the weight of the total composition of N-stearoyl p-amino phenol.

ARNOLD J. MORWAY.  
DAVID W. YOUNG.  
DELMER L. COTTLE.

References Cited in the file of this patent  
UNITED STATES PATENTS

| Number    | Name          | Date          |
|-----------|---------------|---------------|
| 1,659,149 | Niel          | Feb. 14, 1928 |
| 1,789,302 | Callcott      | Jan. 20, 1931 |
| 1,870,074 | Sullivan      | Aug. 2, 1932  |
| 2,604,452 | Morway et al. | July 22, 1952 |